

# United States Patent Office.

WILLIAM SYKES, OF NEWTON LOWER FALLS, MASSACHUSETTS.

*Letters Patent No. 72,563, dated December 24, 1867.*

## IMPROVED MODE OF REMOVING BURRS FROM WOOL.

The Schedule referred to in these Letters Patent and making part of the same.

TO ALL WHOM IT MAY CONCERN:

Be it known that I, WILLIAM SYKES, of Newton Lower Falls, in the county of Middlesex, and State of Massachusetts, have invented a new and improved Process for Removing Burrs and other Vegetable Matter from Wools; and that the following description forms a full and exact specification of the same, wherein I have set forth the nature and principles of my said improvements, by which my invention may be distinguished from all others of a similar class, together with such parts as I claim, and desire to have secured to me by Letters Patent.

This invention relates to a modification and improvement of a process for removing burrs and vegetable matter or substances from wools, for which Letters Patent were granted to me, bearing date July 10, 1866.

The object of the present invention is to save the labor of washing and one drying, which can be done in the manufacture of certain kinds of goods, and to simplify and economize the process formerly patented by me.

The wool is soaked in a solution of sulphuric acid from two to twenty-four hours, (with or without heat,) marking from 2 (two) to 10 (ten) degrees Twaddle's hydrometer, according to the condition of the wool. After the wool is taken from the acid solution and dried, it is then, for the manufacture of certain kinds of goods, dyed direct, which saves the labor of washing and one drying. If the wool be washed in lime or other water after drying, as in the original process, it will of course be suitable stock for any woollen manufacture.

I do not claim broadly the cleaning of wool or depriving it of burrs and other vegetable matter by plunging it in an acidulous solution, for that has been previously patented by me; but

I do claim as new, and desire to secure by Letters Patent—

The immediate dyeing of the wool after the same is taken from the acidulous solution, and either previous to or after the drying of the wool, substantially as set forth.

WILLIAM SYKES.

Witnesses:

LUTHER E. LELAND,  
MOSES GARFIELD.